

Jan. 16, 1934.

H. H. HOLLOWAY

1,943,764

METHOD OF SURFACE TREATMENT OF METAL

Filed Oct. 24, 1931



*Fig. 2.*



*Fig. 3.*



INVENTOR.  
Harry H. Holloway  
BY  
Clarke & Doolittle  
ATTORNEYS.

## UNITED STATES PATENT OFFICE

1,943,764

METHOD OF SURFACE TREATMENT OF  
METALHarry H. Holloway, Apollo, Pa., assignor to Apollo  
Steel Company, Apollo, Pa., a corporation of  
Pennsylvania

Application October 24, 1931. Serial No. 570,800

5 Claims. (Cl. 148—7)

The present invention relates to improvements in the method of finishing metal, and more particularly metal sheets, to produce what is known in the art as a "blue" sheet, having the surface 6 thereof coated with a thin layer of metal oxide of a deep blue color.

Steel sheets of this character are highly desirable in the manufacture of automobile bodies, locomotives, stoves, and the like, wherein the oxidized surface of the sheet forms an efficient 10 guard against rust.

"Blue-annealed" or "steam-blue" steel sheets have been produced heretofore by what is termed the steam process, consisting in passing 15 live steam over cold rolled sheets, which have been re-heated to a certain degree, until they gradually become cooled and assume a blue color by the formation of an oxide coating on the surfaces thereof.

20 The oxide coating resulting from this process has been found to be loosely combined with the sheet, causing the same to crack and flake or chip off when the sheet is subjected to severe bending operations, thus rendering the sheet impracticable for many die-pressed products. Also, the cost of such sheets is materially increased, due to the re-heating operation and the 25 length of time required to complete the process.

My invention contemplates the production of 30 a sheet of the character designated, having an oxidized surface formed in the final rolling or finishing operation by reducing the hot unfinished sheet between cold polished rolls, over which water is continually passed, thereby forming an oxide layer which is both chemically and 35 mechanically combined with the metal of the sheet in such a manner that the metal becomes highly infused or impregnated with the said oxide.

40 The intimate combination produced by my method between the metal and the oxide effectively secures the oxide layer against removal when the sheet is bent, pressed or otherwise worked. In addition, the resulting product has 45 a high finish which successfully masks or removes surface imperfections, and one which is produced without appreciably changing the internal structure of the sheet.

45 In the drawing, which illustrates diagrammatically the apparatus and operation of my invention:

Fig. 1 is an end view of a pair of cold finishing rolls, showing the application of water thereto;

55 Fig. 2 is a fragmentary sectional view greatly

enlarged, taken through a hot metal sheet at the instant of contact with the water and rolls; and

Fig. 3 is a view similar to Fig. 2, showing the sheet after having passed through the rolls.

In the customary method of rolling steel 60 sheets, the sheet bar is first hot rolled to about 60% of length, pickled, hot rolled to size and gauge, and then sheared into sheets of the required shape and dimension.

They are next either box-annealed or nor- 65 malized, depending upon the desired internal structure of the sheets, cooled, pickled, and then cold rolled through the required number of passes with the sheets and rolls cold and dry, to bring them down to the exact gauge and to pro- 70 duce a hard smooth finish. Steel sheets produced by this method are steel gray in color.

In producing "blue" sheets of the character described by means of my method, the above operations are followed up through and including 75 the shearing of the sized sheets, and then they are pickled in the usual solution and by any suitable process.

The sheets are then heated, preferably in a continuous furnace or by box-annealing, until 80 they are raised to a temperature of 500-1500 degrees Fahrenheit. This temperature range may vary for various alloy sheets, depending upon the nature of the alloy. For example, for the usual steel automobile body sheets, it has 85 been found that the best temperature is 1200 degrees Fahrenheit to give the most satisfactory results.

The hot sheets are then taken to a finish mill 90 comprising a pair of cold polished rolls 2, set to accurately reduce the sheets to the required gauge. The said rolls are flooded with water in the manner shown, by means of perforated pipes 3 or other suitable means, for completely covering the roll surfaces with the water, which is preferably cold.

Each sheet A is preferably aerated by rotating or otherwise exposing the same to atmospheric action before passing to the rolls 2, to 100 free the surfaces thereof from foreign matter and to tend to equalize the surface temperatures on both sides of the sheet.

The sheet A is then drawn through the cold 105 wet rolls 2 at the said prescribed temperature. The intense heat of the sheet converts the water into steam at the instant of contact, which steam is confined in the minute space between the rolls and the surfaces of the sheet. The oxygen in the steam chemically combines with the metal 110

of the sheet to produce a film or layer of oxide 4 covering the surfaces of the sheet.

Prior to its passage through the rolls 2, the sheet ordinarily has imperfect surfaces, due to 5 the presence of a large number of minute defects or abrasions such as blow holes, pin holes, scratches, pits, etc., resulting from the reducing operations. Such imperfections are indicated at 5 in Fig. 2, greatly enlarged.

10 At the instant of contact of the hot sheet with the water and rolls, the film or layers of oxide 4 produced will be in such a state of fluidity that they will fill the imperfections or openings 5, as indicated in Fig. 2.

15 The instantaneous mechanical action or pressure of the rolls 2 operates to roll the oxide layers 4 into the surfaces of the sheet A. Due to the reduction of the sheet A in passing through the rolls, the surfaces of the sheet and 20 the oxide layers will be highly compressed and rolled together, thereby forming a mechanical combination between the sheet and the oxide layers by the deformation and depression of the oxide-containing imperfections or openings 5, as indicated in Fig. 3.

25 The hard smooth surfaces of the finishing rolls will produce a continuous smooth finish on the oxide coatings or layers which will be practically free from abrasions of the character described 30 and for which sheets may be rejected as imperfect. In addition, when the sheet has cooled, the oxide will take on a dark blue color.

35 Actual tests have shown that the oxide coatings so formed will not crack or flake off when the sheet is subjected to the most severe bending actions, as, for example, bending the sheet back upon itself. Also, steel sheets produced by means of my process are being satisfactorily 40 used in the production of die-pressed automobile bodies, or other deformed shapes.

45 Thus, it will be seen that by means of my method, a "blue" sheet may be produced having all the desirable characteristics of the old "blue-annealed" sheet, with the added property that the oxide coating will not come off during the working of the sheet. And, further, the re-heating operation of the "steam-blue" process 50 is dispensed with, thereby decreasing the time element as well as the actual cost of heating. Time is also saved, due to the fact that it is not necessary to cool the sheets as in the old process before cold rolling and finishing.

An important application of my invention re-

sides in the use of the process in re-claiming and perfecting cold rolled sheets which have been produced under the old method and have been rejected for surface defects remaining after having passed through the final cold rolling operation.

80

The sheets are heated to the desired temperature within the prescribed range, and then passed through the cold wet rolls as stated, to apply the oxide coating and produce "blue" 85 sheets wherein the surface defects are successfully masked or removed, due to the combined action hereinbefore described.

I claim:

1. The final step in the method of finishing 90 steel sheets consisting in applying an oxidizing blue finish to the opposite sides of thin previously densified steel sheets by re-heating the sheet, then passing it between a pair of polished rolls each supplied with an individual water film, and effecting instantaneous oxidation and compression of the resulting oxide upon and into opposite sides of the sheet throughout their surface areas.

95

2. The final step in the method of finishing 100 steel sheets consisting in applying an oxidizing blue finish to the opposite sides of thin previously densified steel sheets by re-heating the sheet, then passing it between a pair of polished rolls each supplied with an individual water film, and effecting instantaneous oxidation and compression of the resulting oxide upon and into the 105 plane and other surfaces on opposite sides of the sheet throughout their surface areas.

105

3. The final step in the method of finishing 110 steel sheets which consists in forming a permanent blue oxide coating on the surfaces thereof by passing said sheets while heated, between a pair of cold polished rolls each supplied with a water film.

115

4. The method of reclaiming and refinishing 120 cold rolled steel sheets having surface defects which consists in reheating the sheet, and forming a permanent blue oxide coating on the surfaces thereof by passing said sheet between a pair of cold polished rolls each supplied with a water film.

120

5. As an article of manufacture, a steel sheet, 125 the surfaces of which contain a permanent blue oxide coating formed by subjecting the sheet while heated to the simultaneous action of cold polished rolls and water.

HARRY H. HOLLOWAY.

55

130

60

135

65

140

70

145

75

150